

Feb. 6, 1940.

W. A. WISSLER

2,189,387

## METHOD OF MAKING HARD COMPOSITIONS

Filed March 5, 1938



*Pig. 2*



Fig. 3



INVENTOR  
WILLIAM A. WISSLER  
BY  
*Ed Greenwald*  
ATTORNEY

## UNITED STATES PATENT OFFICE

2,189,387

## METHOD OF MAKING HARD COMPOSITIONS

William A. Wissler, Niagara Falls, N. Y., assignor  
to Haynes Stellite Company, a corporation of  
Indiana

Application March 5, 1938, Serial No. 194,109

1 Claim. (Cl. 75—137)

This invention relates to the production of cast hard compounds of difficultly fusible metals, and compositions containing such compounds.

To produce hard, strong casings of the carbides or other hard compounds of difficultly fusible metals, or of alloys containing such compounds, mixtures of the desired ingredients are ordinarily melted and the fused products rapidly solidified in molds and rapidly cooled directly after their solidification. The methods of melting and cooling heretofore in use involve the melting of small individual batches of compound, or the constituents thereof, in a crucible. The extremely high temperature required to melt the compounds limits the amount of material that can expediently be melted in any one batch by these methods and also causes excessive burning or scoring of the molds and crucibles. Ordinarily, a mold or crucible can be used only once, or at most only a few times. Further, such molds and crucibles usually consist of carbon and at the high temperatures involved the melt tends to pick up a substantial proportion of this element. Inasmuch as the carbon content of the cast hard compound must be within certain well defined limits to obtain a material of optimum physical properties much of the cast compound produced by the methods heretofore in use is often unsatisfactory.

An object of this invention is to provide a continuous or semi-continuous process, free from the disadvantages mentioned above, for the production of cast carbides, borides, silicides, nitrides, and other hard compounds, of the difficultly fusible metals of the fourth, fifth, and sixth groups of the Mendelejeff periodic arrangement of the elements, with or without auxiliary metals such as iron, cobalt, and nickel. Another object is to provide apparatus suitable for use in practicing the process of the invention. A further object is to provide cast compounds of the class defined above in the form of elongated pellets.

These and other objects are attained in the process of the present invention which comprises preparing bonded mixtures of the desired ingredients and melting and cooling said mixtures in the manner explained below.

The invention will be described in connection with the attached drawing, in which:

Fig. 1 is a sectional schematic view of a form of an apparatus embodying the invention; and

Figs. 2 and 3 are sectional schematic views of alternative forms of the apparatus shown in Fig. 1.

In the production of cast hard compounds by a continuous process of the invention employing

the form of the apparatus shown in Fig. 1, a mix 27, consisting of the desired ingredients, suitably in comminuted form, in the desired proportions together with a carbonaceous binder such as pitch, glue, or oil, or other binder, is placed in a mixing chamber 24 which suitably comprises a continuous screw 25, a die 23 having a plurality of small holes, and a second die 26 having a single opening preferably centrally located. The chamber 24 may, if desired be heated, in any suitable manner, to lower the viscosity of the bonding materials of the mix, thus ensuring a more intimate mixture between the comminuted dry ingredients and the bonding materials. The bonded mix 27 essentially contains at least one of the difficultly fusible metals of the fourth, fifth, and sixth groups of the periodic system, for example, chromium, molybdenum, tungsten, titanium, zirconium, vanadium, columbium, or tantalum, or compounds of such metals, and at least one of the hard compound forming elements such as carbon, boron, or silicon, or nitrogen, or compounds of said elements, with or without one or more auxiliary metals such as iron, cobalt, and nickel.

The bonded mix 27 is forced, by means of the screw 25, through the die 23 and the die 26 into and through a baking furnace 22, from which it emerges as a solid coherent mass or rod 11. The baking furnace is heated by an electric resistance 28 or by other appropriate means.

The rod 11 is connected as one electrode in an electrical circuit, and an electrode 12, preferably of carbon or graphite, is connected as the other electrode. Inasmuch as the process is continuous, the electrical connection may be made to the rod 35 11 by suitable contact with the mix 27 at a point near the baking furnace 22. Preferably, the rod 11 is made the positive electrode, and the carbon 12 the negative electrode, but the polarity of the two electrodes may be reversed or an alternating 40 current may be substituted for a direct current. The electrode 12 may be held by an electrode holding and feeding device 14 of any desired type to establish and maintain an electric arc 10 of constant length and of sufficient intensity to melt 45 the electrode 11. A cover 15 may be provided, if desired containing openings for the insertion of the electrodes and for the insertion of a tube 20 through which an inert or reducing gas, such as hydrogen or nitrogen, may be introduced. The 50 cover 15 preferably consists of a non-conducting material; if the cover is a conducting material, it should be insulated from the electrode. The cover 15 and the electrode holding and feeding device 14 are supported on a platform 16 provided with an 55

opening 17 through which compound melted by the heat of the arc 10, in the form of individual elongated pellets 19, is discharged by gravity into a receptacle 18 located under the opening 17 and 5 containing a quenching medium 21 such as oil, water, gas, or molten salt. The pellets 19 do not agglomerate or cohere, and they may be removed from the quenching medium without interrupting the melting operation. If desired, the pellets of 10 cast compound may be cooled by other means, for example, by air cooling or by permitting the compound to remain in close proximity to a colder solid body.

In the production of cast hard compounds employing the alternative form of apparatus shown in Fig. 2, the rod 11 is prepared independently of the melting operation, and is melted in the simplified apparatus shown. The various parts of the apparatus of Fig. 2 are designated by numerals 20 corresponding to those of Fig. 1 so that the description of melting and quenching given in connection with Fig. 1 applies, in a like manner, to Fig. 2.

In the production of cast hard compounds employing the form of the apparatus shown in Fig. 3, the rod 11, which may be prepared either as described in connection with Fig. 1 or independently of the melting and quenching operations, is melted by the heat of an electric arc 30 formed between carbonaceous electrodes 12. The method of quenching the melted compound is the same as that described in connection with Fig. 1. The form of the apparatus shown in Fig. 3 is especially applicable to the melting of bonded rods which are substantially non-conducting, for example, rods bonded with soluble silicate bonding materials such as sodium silicate.

Alternatively a conductive composite rod similar in composition to the rod 11 may be substituted for the carbon electrode 12 in any of the forms of the apparatus and process described above.

A typical procedure for the production of cast tungsten carbide, employing the form of apparatus shown in Fig. 2, is as follows:

A pulverized mixture consisting of:

|                             |     |      |
|-----------------------------|-----|------|
| Tungsten carbide (2.58% C.) | gm. | 2400 |
| Cobalt                      | gm. | 24   |
| Carbon                      | gm. | 12   |
| 50 Pitch                    | gm. | 184  |
| Oil                         | cc. | 40   |

was heated and formed into a plastic mass and extruded, while hot, into a composite rod five-sixteenths of an inch in diameter. The rod was then baked to convert the pitch into coke and to form a solidly cohering mass. An arc was formed between the composite rod connected as the positive electrode, and a graphite rod connected as the negative electrode, in a direct current circuit. A current of about 200 to 250 amperes was used. As the composite metal rod melted, the molten material, in the form of individual elongated drops or pellets, was imme-

diately discharged by gravity into a receptacle containing water. A chemical analysis of the cast tungsten carbide and cobalt composition so produced revealed that it contained 3.6% carbon, which is approximately the carbon content 5 required for optimum physical properties in a cast hard compound of this type. Furthermore, a recovery of 88% of the weight of the bonded rod consumed in the electric arc was obtained.

According to other embodiments of the invention, bonded rods are melted by high temperature heat produced, for instance, by an atomic hydrogen arc; or by the combustion of gases. It will be appreciated that the specific examples of melting are given herein by way 15 of illustration, and the present invention is not limited to or by such examples. Although I have described the production of cast tungsten carbide alloy as an example, it is within the invention to produce carbides, borides, silicides, nitrides, or other hard compounds of any of the 20 difficultly fusible metals such as chromium, molybdenum, tungsten, vanadium, columbium, tantalum, titanium, or zirconium, or alloys containing such hard compounds.

By the method of the present invention, crucibles, molds, and other expensive refractories heretofore used in the production of cast hard compounds are eliminated. Also, the recovery 25 of cast compound in relation to the amount of composite rod melted is comparatively high. Further, the carbon content of the compound may readily be held within the narrow composition limits necessary to produce a cast hard compound of optimum physical properties. The 30 method of the present invention may be made either continuous or semi-continuous, thus permitting greater flexibility in the production of cast hard compounds than heretofore available.

Cast hard compounds produced in accordance 40 with the invention are ordinarily in the form of elongated pellets which are substantially homogeneous in structure and composition. Such pellets are suitable for use as hard facing material for tools, or in other applications where 45 high resistance to wear and abrasion is one of the requisites of the material. They may readily be applied to metal surfaces by welding, either electric or oxy-acetylene, or by any other well known methods. If desired, the pellets may be 50 enclosed in a metal sheath, or bonded with a suitable binder, and advantageously employed in this manner as hard facing welding rods.

I claim:

A method of producing cast compositions of 55 the class described which comprises mixing the ingredients thereof with a binder; forming said bonded mixture into a solid rod; melting said rod by the heat of an electric arc formed between said rod and a carbonaceous electrode, and 60 promptly discharging the fused composition by gravity into a cooling medium.

WILLIAM A. WISSLER.